

## UNITED STATES PATENT OFFICE

CARLETON B. EDWARDS, OF INDIANAPOLIS, INDIANA, ASSIGNOR TO PETER C. REILLY,  
OF INDIANAPOLIS, INDIANA

## PROCESS OF CARBURIZING AND CARBURIZING COMPOSITION

No Drawing. Application filed April 29, 1927, Serial No. 187,706. Renewed December 9, 1930.

This invention relates to the case-hardening or carburizing of steel articles in the presence of a substantially non-burning carburizing composition and to the preparation of this material.

Steel articles are usually case-hardened or carburized by the hot dump process at temperatures varying between 1550° to 1700° F. (843° to 927° C.). It has become the standard practice to quench certain carburized articles directly from the furnace at the carburizing temperature. For example, in box packing, the contents of the boxes are dumped onto a screen, the steel articles passing into a quenching medium, and the carburizing composition dropping through the screen into cars or onto the floor, where it is allowed to burn or is subjected to a water bath. It is general rotary tube furnace carburizing practice to directly quench in the manner referred to.

In the operation of the direct quench carburizing process, as set forth, it has been customary to use a carburizing composition which burns or ashes. In some plants it is quite common for the hot carburizing material, after use in the carburizing step, to burn and ash for several days. When this is allowed, before the carburizing material can be reused, it is often necessary to add fresh material, averaging in many cases as high as 50%. As an alternative procedure, instead of allowing the carburizer to burn and ash, it is subjected to a water quenching but this is unsatisfactory due to the washing away of the soluble activators present in the carburizer. Further, the carburizer must be dried before it is satisfactory for reuse.

The carburizer burns and ashes for several days due to its inherent characteristic of combusting rapidly on being dumped red hot from the carburizing pots or furnaces. This burning and ashing results in a notable wastage of the carburizing material. The rapid combustion of the carburizing material or composition is due, in a great measure, to its high porosity and its low ignition temperature. Further, the rapid combustion is influenced by the ash and volatile content of the carburizing material.

The common carburizing compositions are, in general, composed of such materials as wood charcoal, gas coke or petroleum coke containing chemical energizers bound on to the particles with molasses or equivalent binders, or soaked into the particles. Coal and energizers may also be made into pellets and heated to coke the coal. Charcoal products are especially characterized by a rapid combustion. The carburizing composition made by coking coal and an activator also possesses rapid combusting qualities, due largely to the high porosity of the coked mass, its low ignition temperature, the oxygen always present in coal, and the large amount of coal ash and volatile matter. The high porosity is probably due principally to the rapid coking of the coal in the presence of a relatively large quantity of an activator and ash functioning to separate the carbon particles, and to present an enormous surface area favoring rapid combustion when the used carburizing material is dumped hot from the boxes or pots.

The present invention has for one of its objects the case-hardening or carburizing of iron and steel articles by a hot process in the presence of a carburizing composition characterized by the property of becoming extinguished without appreciable burning or ashing when it is poured, after use in the carburizing step, red hot from the carburizing boxes or furnaces.

It is a further object of this invention to produce a carburizing composition that is substantially free from porosity, so low in combustibility that it cools below its ignition temperature readily in air and, at the same time has the following qualities which are needed for the best results and greatest economies in steel carburization, namely, low volumetric and weight loss on first use, low ash, sulfur and volatile content, high ignition temperature, comparatively low weight per cubic foot contrasting notably with some of the carburizing compositions now used, high strength of particle, and low specific heat.

Having conceived the desirability of hot carburizing in the presence of a substantially non-burning carburizing material, it follows

that the next step is to produce this material. The solution of this problem involves as one of its elements the selection of the raw carbonaceous material. One of the best raw materials is coal tar carbon produced in accordance with the disclosure in U. S. Patent No. 1,230,782, to Reilly. This material is low in ash and sulfur content. However, any other carbon base may be used which is sufficiently pure and which, when thoroughly baked, has a low porosity, a relatively high ignition temperature and is substantially non-burning in air at the temperature used in hot carburizing. For example, certain petroleum cokes may be used as the carbonaceous base, providing their properties, including freedom from ash and sulfur, come within the specifications referred to. It is desired to indicate that while the preferred material is the coal tar carbon referred to, broadly the invention contemplates the use of any carbonaceous base having the desired properties which have been briefly referred to, and will be later more specifically indicated.

25. Specifically, a suitable carbonaceous base is one having a sulfur content between 10% and .40% and an ash content between .15% and 2.0%, the latter, of course, being exclusive of the ash content of any added energizers such as carbonates.

While the selection of the raw carbonaceous material is of prime importance, it is of equal importance to carbonize the raw material under proper conditions. It is possible to carbonize coal tar having low ash and sulfur content so that it has a high porosity and will burn readily when used in a hot carburizing process. Such carbonizing is to be avoided; the operation is to be carried out under such conditions as produce a substantially non-burning product. In order to produce a non-burning product, it is necessary to carbonize slowly with but little inorganic material present and bake at a temperature between 600° and 850° C. It is of real importance to have little inorganic matter present during the carbonizing step as small amounts of some inorganic products act as catalytic agents functioning to lower the ignition temperature and increase the combustibility of the finished carburizing material, which, of course, is to be avoided. While in general the latter is true, I have found that some substances, for example sodium carbonate, increase the strength and hardness of the carbonized mass, which is desirable in rotary carburizing work. Further, the purity of the carbon base including its freedom from ash, not only causes lower combustibility, but also gives a longer life to the carburizing composition, since there is no ash to neutralize activators by forming silicates and other compounds.

60. In general, the carbonizing process should be carried out slowly and at the correct temperature so that most of the volatile matter will be driven off and simultaneously there

will be little tendency to form a material of high porosity.

The method of manufacture of a substantially non-burning carburizing composition is as follows:

A carbonaceous base having a low sulfur and ash content for example, Reilly carbon is mixed with chemical energizers. Satisfactory results are obtained by using either of the following mixes, although, it is, of course, understood that the same may be varied.

|                   | Per cent | Per cent |
|-------------------|----------|----------|
| Reilly carbon     | 60       | 50       |
| Sodium carbonate  | 1.5      | 4        |
| Barium carbonate  | 7.5      | 12       |
| Calcium carbonate | 1.5      | 6        |

The carbon in either of the above mixes is in the form of small sized particles preferably between two and twenty mesh. The mix is made into carburizing particles to which is added a hard pitch melting at a suitable temperature, preferably around 200° C. Pitches may be used having melting or softening points varying between 140° C. and 325° C. Coal tar pitch is the most suitable coating agent. However, petroleum pitch, wood tar pitch and vegetable oil pitch may be used if they have a low ash and sulfur content. In the above examples the addition of 29.5% and 28% respectively of pitch gives good results.

After the particles of raw carburizing material have been coated the entire mix is charged into a rotary kiln. The mix is carburized slowly at a temperature varying between 600° and 850° C. the final temperature being close to the latter to produce a good hard particle. It is important that the passage of the mix through the kiln be regulated so that the baking operation is not performed too quickly. Using a kiln about twenty to thirty feet long, the time of passage should approximately be between 10 and 15 minutes. The baking is to be carried out so as to produce a carburizing composition having a volatile content between 2% and 12%, and of low specific heat.

The carburizing compound may also be made by incorporating the energizer in coal tar or coal tar pitch and coking the mass, or by causing the energizers to adhere to the carbon by binders, any of these methods being so carried out that the porosity of the material is so low, and the ignition temperature so high, that the material ceases to burn materially when dumped hot.

The product resulting from the proper choice of raw materials and a regulated baking action may be termed a non-burning material since it does not burn appreciably upon exposure to air after use in the carburizing step, does not ash enough to be visible under ordinary conditions of use, and therefore, for all practical purposes, is non-burning.

The carburizing material resulting from

the treatment set forth has an ignition temperature varying between 460° C. and 550° C. and is very difficultly combustible when dumped red hot. This is due to the low 5 porosity of the carbon as compared to charcoal, to the purity of the carbon, including its freedom from oxygen and ash, and to its very high ignition temperature after the baking out process. The material when 10 dumped becomes extinguished readily and the loss by burning is relatively small, varying, for example, between 0.3% and 1.8%. In general, it may be stated that the burning 15 loss on hot dumping is usually under 0.5% under conditions where using the usual carburizing material, there is a loss averaging about 10% but which may vary between 5% and 38%.

When using the substantially non-burning 20 carburizing material, it is found that the addition of 5% to 20% of new material keeps up the volume and carburizing activity, even under hot dumping conditions. Due to the 25 method of baking employed including the employment of a relatively high temperature, the original volatile loss on a first run carburizing operation is from 2% to 12% instead of 15% to 40% when using carburizing 30 compositions not produced in accordance with the method set forth.

Utilizing the non-burning carburizing material, the case-hardening or carburizing of steel articles by the direct-quench process may be carried out with an enormous saving 35 of the case-hardening or carburizing composition. Further, the process may be carried out without quenching the carburizing material after use, thereby permitting the economical employment of soluble activators 40 in the carburizer. Ordinarily, if these are present in the burning type of carburizing material, they are lost, when the material is subjected to a water-quenching to extinguish the carburizer.

45 The differences existing between the non-burning type of carburizing composition and the charcoal-coke products and coal and activator coked masses, are:

1. Upon dumping in the air at red heat, 50 the non-burning product becomes extinguished without burning—whereas the others continue to glow, as does charcoal, and may ash completely. The following data are 55 illustrative: Non-burning type product shows 0.4% to 1.8% burning loss; others under similar conditions 5.2% to 37.7%.

2. The non-burning carburizing composition is black or grey, carbon color—after direct quench. Other products show the white 60 ash resulting from substantially complete or partial combustion.

3. In order to show the marked difference 65 between the non-burning composition and other products, place the former and either a charcoal compound or coal pellets side by

side, on a wire screen. Then place a burner below and heat to red heat. Remove the flame. The non-burning product darkens, ceases burning rapidly, and shows no ash. The other continues to glow, shows white ash 70 and in many cases ashes completely.

4. At a given temperature, for example, 500° C. the non-burning product burns much more slowly (does not glow). Another way 75 of stating this is, it requires a higher temperature to give the same degree of glowing or burning.

5. In one series of tests, equal quantities of several materials were heated to a carburizing temperature (1650° F.) and dumped hot. 80 The burning loss on the non-burning product was 0.4% to 1.1% as against a range for the others of from 9.5% to 37.7%. Under different conditions of test these values will be different, but of the same relative order. 85 These are merely indicative of the difference between the non-burning product and others, showing more clearly how and why such improvement and economies are shown by non-burning material in actual plant usage. 90

6. Another experiment showing similar results was carried out as follows: Carburizing particles of various kinds were heated in a flame to between 800° and 900° C. The flame was then removed and the particles blown by 95 the breath or a stream of air. All of the compositions glowed brightly with the exception of the non-burning material which was quickly extinguished by the air current.

7. Actual ignition temperatures were determined by placing several particles of a carburizing composition in a glass tube in an electric furnace, carrying the furnace tube and composition to a given temperature and passing a stream of air over the material. 100 The ignition point was taken as the lowest temperature at which the particles would glow when the air was passed over them. The non-burning composition first showed 105 glowing at 475° C. to 550° C. (different samples). The others glowed between 325° and 415° C. under similar conditions. It therefore appears that a temperature of 450° C. is well above the ignition point of any carburizing composition heretofore used, where- 110 as the same temperature is below the ignition point of the non-burning composition. The non-burning carburizing composition is characterized by an ignition temperature of above 450° and this characteristic distinguishes the 115 new product from compositions heretofore used.

8. A more definite test showing the difference in combustibility, which is the principal cause of the non-burning quality of my product, was carried out as follows: After the ignition point had been found as described above and one or more particles were glowing nicely, the glass tube containing the material 125 was removed from the furnace but the same 130

stream of air was continued. In the case of all compounds other than the non-burning type, the particles continued to glow and ash after they were removed from the external source of heat. The non-burning type, however, even though glowing when removed, rapidly dropped in temperature and became black almost at once. The difference here, of course, is due to the lower rate of burning in the case of the non-burning type. Its combustion under these conditions is insufficient to keep the particle up to or above its ignition point. The combustibility being lower than other carburizing compounds and the ignition temperature being higher, both contribute to the production of a carburizing composition admirably suited for carburizing economically by a hot process.

In practically all hot dump procedures the steel and carburizing material are emptied from the furnace or pots at from 1550° to 1800° F. (843° to 982° C.) which is considerably above the ignition point of any of the carburizing compositions. Therefore, when a carburizing composition is poured into the air at this temperature, ease of burning, the porosity of the composition and the ignition temperature in air, are all contending factors causing the composition to be substantially non-burning. While porosity is a very important factor, it is not the only cause of a high burning rate and long continued burning in air. Small amounts of certain catalytic agents will function to lower the ignition temperature and increase the combustibility of carbonaceous materials. In general, it may be stated that in a non-burning carburizing composition, the presence of impure carbon, porous carbon, easily burning carbon and oxides, particularly oxides of lead, should be avoided. This may be expressed a little differently by stating that the raw materials should be so selected and the process of treatment so carried out, as has been indicated in illustrated examples, to produce an allotropic modification of carbon which does not burn.

Summarizing, it may be stated that the new product is characterized by the following properties:

1. Its volatile content varies between 2% and 12% instead of 15% and 40% as in products heretofore used. This lower weight loss results in great economy.
2. It possesses high heat conductivity.
3. The ash content exclusive of carbonate is between 1.5% and 2.0%. In compositions heretofore used, the ash content has varied between 5% and 10%. Low ash means little fusion of the activators with the ash thereby preventing loss in carburizing efficiency.
4. The sulfur content varies between .10% and .40%.
5. It has a low specific heat (approximately .3%). Being baked more thoroughly and

being low in ash, the material is more nearly pure carbon and consequently has a low specific heat.

6. The volume loss, first run, averages between 3% and 14% as against 16% and 40% loss in the compositions heretofore used. 70

7. The weight loss, first run, averages between 2% and 12% exclusive of moisture as against 15% and 40% in the compositions heretofore used. 75

8. The finished non-burning carburizing material has a low weight per cubic foot. Specifically, this weight varies between 24 to 36 pounds per cubic foot, contrasting notably with some of the carburizing compositions now used, which usually weigh approximately 44 pounds per cubic foot. 80

9. The strength of the non-burning carburizing particles is such as to favorably resist wear and crushing in use. The particle is hard and firm; much more so than charcoal products, which are severely ground in the rotary carburizing furnace. 85

The non-burning carburizing composition herein set forth may be provided with a non-carburizing shell or coating, preferably of carbon, which serves as an insulator to prevent contact between the materials in the shell and the article being carburized. 90

By the term "iron articles" as used in the specification and claims, it is intended to include articles made from iron, steel, and iron and steel alloys. 95

By the term "non-burning carburizing composition" as used in the specification and claims, it is intended to define a composition which does not ash enough to be visible, and appreciably burn upon exposure to air after use in a carburizing operation carried out at a relatively high temperature. 100

I claim:

1. As a new article of manufacture a substantially non-burning carburizing composition having as an essential element a predominating quantity of substantially non-porous carbon. 110

2. As a new article of manufacture a substantially non-burning carburizing composition consisting mainly of a substantially non-porous carbon of low combustibility and having a volatile content averaging between 2% and 12%. 115

3. As a new article of manufacture a substantially non-burning carburizing composition having as an essential element a predominating quantity of a substantially non-porous carbon of low combustibility and having a volatile content averaging between 2% and 12% and characterized by the property 120 of self extinguishment.

4. As a new article of manufacture, a substantially non-burning carburizing composition having as an essential element a predominating quantity of substantially non- 125

porous carbon and likewise containing a chemical energizer.

5. As a new article of manufacture, a substantially non-burning carburizing composition having as an essential element a predominating quantity of substantially non-porous carbon and likewise containing an energizer.

In testimony whereof I have signed my  
10 name to this specification.

CARLETON B. EDWARDS.

15

20

25

30

35

40

45

50

55

60

65